# EUROPEAN PATENT SPECIFICATION

(11) **EP 0 293 119 B1**
(45) Date of publication and mention of the grant of the patent: **19.08.1992**
(21) Application number: 88304405.9
(22) Date of filing: 16.05.1988
(51) Int. Cl.: D21H 17/62, D21H 17/71

(54) **Paper sizing compositions**
Zusammensetzungen zum Leimen von Papier
Compositions de collage pour papier

(30) Priority: 26.05.1987 GB 8712370
(43) Date of publication of application: 30.11.1988
(73) Proprietor: Eka Nobel Landskrona AB, S-261 23 Landskrona (SE)
(72) Inventor: Bussell, William Robert, Bristol BS13 0AH (GB); Morgan, Nicholas Stuart, Bristol BS5 9DJ (GB)
(74) Representative: Schöld, Zaid

(56) References cited:
- EP-A- 0 018 007
- WO-A-86/02677
- GB-A- 851 187
- GB-B- 1 444 751
- US-A- 2 138 325
- US-A- 3 817 768
- US-A- 4 025 354
- US-A- 4 522 686
- NOTES OF THE TECHNICAL ASSOCIATION OF THE PULP AND PAPER INDUSTRY, 1983 SIZING SEMINAR, Savannah, GA, 16th-18th November 1983, pages 61-65, Tappi Press, Atlanta, GA, US; D.R. DILL: "Dispersed rosin sizes: why and how"

## Description

This invention relates to paper sizing compositions, methods for making such compositions, processes for sizing paper products using these compositions and paper products which have been sized with these compositions.

Stable dispersions of rosin or rosin-based products are well-known and have long been used, especially as sizing agents in the manufacture of paper. In this specification, the term "paper" is used, for convenience, to mean all forms of paper, paperboard and related products whose manufacture involves the employment of a sizing agent upon cellulosic or other fibres. Paper sizing agents are usually employed either by being added to the cellulosic or other fibre stock from which a web is later made or by being applied to the surface after the web has been formed. Rosin-based sizing agents depend for their sizing effect upon the formation of electrostatic bonds between the sizing agent and the cellulosic or other fibres of the paper stock or web. Highly efficient sizing agents have been developed more recently which includes many kinds which, in use, form chemical bonds and these are thus known as "reactive" sizing agents. A major development in the paper-making size art was the discovery that reaction products formed by rosin or unsaturated compounds present in rosin, on the one hand, and unsaturated carboxylic acids or their anhydrides, especially maleic or fumaric acid or maleic anhydride, on the other hand, have greatly enhanced sizing efficiency, as compared with those kinds of sizing agents which are essentially dispersions of rosin itself. These so-called "maleated" rosin reaction products and other related sizing agents are rather expensive to make and so they are often used to fortify conventional rosin dispersions, rather than to replace them. This is done by adding a quantity of a "maleated" rosin reaction product to a conventional rosin dispersion and the resultant compositions are commonly known as "fortified sizing agents".

In practice, all types of paper sizing agents are usually in the form of stable dispersions and they cause sizing by depositing rosin-based or other materials on to the fibre stock or the paper web, so that sizing essentially involves breaking the stable dispersion. This can occur on contact between the dispersion and the stock or web, where the latter is effective to destroy the stability of the dispersion. Usually, however, adequate sizing does not arise from mere contact of the paper sizing agent with the paper stock or web. Instead, it requires the presence of a co-reactant to break the dispersion and so cause the desired deposition of sizing components on the fibres of the paper stock or web. The most commonly employed co-reactants are aluminium compounds and, especially, aluminium sulphate, papermaker's alum and the polyaluminium chlorides.

The majority of paper-making processes involve the separate addition or application of the rosin-based size and a co-reactant to the paper stock or the paper web. There have been proposals, notably those in U.K. Patent Applications 2050453A and 2159183A and U.S. Patent 4522686, to prepare sizing compositions comprising both a rosin component and a suitable reactant, which compositions offer the advantage of sizing using a single composition, but these have not been entirely successful, either because the dispersions are unstable or because their effectiveness as a size has been reduced. For whatever reason, the majority of paper mills utilise a sizing process which involves the use of two separate components, despite the inherent difficulties involved.

US Patent 4522686 and International Application WO 86/02677 discloses rosin dispersions which rely for their stability on the formation of a coating of a cationic polymer around the rosin particles of the dispersion which is thus cationic and remains stable through mutual repulsion of postive charges.

It has been discovered that dispersions, comprising a rosin component and an amine salt of a rosin acid, which are stable and which impart excellent sizing properties to paper, can be prepared by the incorporation of at least one aluminium compound into a composition of a rosin size and an amine salt of a rosin acid.

According to one aspect of the present invention, there is provided a paper sizing composition in the form of a preformed stable aqueous dispersion for subsequent use in a paper-sizing process, characterised in that the composition has the ability to size paper stock, sheet or web to an effective extent when brought into contact with the stock, sheet or web during the sizing process and comprises the material obtainable by addition of at least one aluminium compound to an aqueous dispersion comprising rosin size and an amine salt of a rosin acid.

The invention also provides a method of manufacture of a paper-sizing composition, the composition being characterised in that it is in the form of a stable aqueous dispersion for subsequent use in a paper-sizing process and has the ability to size paper stock, sheet or web to an effective extent when brought into contact with the stock, sheet or web during the sizing process, the method comprising first forming an aqueous dispersion comprising rosin size and an amine salt of a rosin acid and then introducing at least one aluminium compound into the dispersion; and a process of manufacture of a sized paper product, wherein a paper-sizing composition is added to fibre stock which is then made into paper or is applied as a surface size to a prepared paper web or sheet, the composition being characterised in that it comprises the material obtainable by addition of at least one aluminium compound to an aqueous dispersion comprising rosing size and an amine salt of a rosin acid.

Rosin is a solid resinous material which occurs naturally in the oleoresin of pine trees. It is obtained from one of three main sources, the oleoresin exudate of living pine trees, the oleoresin contained in the aged stumps of pine trees and from the tall oil produced as a by-product in the kraft paper industry. Rosin is a complex mixture of cyclic terpene carboxylic acids together with a small amount of non-acidic components. A major constituent of rosin is the tricyclic doubly unsaturated mono-carboxylic acid, abietic acid.

Abietic acid undergoes Diels-Alder addition with dienophiles. Rosin may therefore be reacted with dienophilic carboxylic acids such as maleic acid, maleic anhydride or fumaric acid to form a tetracyclic polycarboxylic acid. This reaction with these dienophiles is commonly termed fortification. The product of such reaction between rosin and a dienophile is commonly termed a fortified rosin. Fortified rosin dispersions are used as sizing compositions in the paper sizing industry and the novel dispersions of this invention may comprise either rosin or fortified rosin or a mixture of the two. The rosin may have been treated with formaldehyde in order to enhance their stability. Esterified or disproportionated rosins may also be used in the compositions of this invention. Esterified rosins are rosins which have been reacted with an alcohol which is preferably a polyol such as glycerol. Disproportionated rosins are rosins which have been treated by a catalytic process in order to improve their stability to oxidation. Mixtures of any of these types of rosin may be used in the compositions of this invention.

The preferred rosin for use in the composition of this invention are fortified rosins. The preferred fortified rosins are those wherein the rosin has been reacted with from 5 to 50% of its own weight and generally about 10% by weight of a dienophile. Such rosins comprise a mixture of fortified and unfortified rosin. The two are normally used in combination in view of the fortification which would render the use of a product comprising fortified rosin only prohibitively expensive. The most preferred type of rosin is fortified tall oil rosin.

The amine salt of the rosin acid may be produced by the neutralisation of any of the rosin or rosin derivatives described above. It may be prepared separately and added to the rosin dispersion, but more usually it will be produced in situ by the addition of sufficient amine to bring about the partial neturalisation of the acid content of the rosin. Thus in a preferred embodiment the amine salt is the salt of the rosin acid or acids present in the rosin component of the dispersions of this invention.

The salt of the rosin acid may be produced by neutralising the acid either prior to or after its conversion to a rosin derivative. The neutralisation may be carried out using an amine having the formula:
wherein substituents R₁, R₂ and R₃, which may be the same or different, represent alkyl or alkenyl groups comprising from 1 to 4 carbon atoms or a hydrogen atom, with the proviso that at least one of the substituent is not a hydrogen atom. Preferably at least two of the substituents groups R₁, R₂ and R₃ represent alkyl groups and, most preferably, all three of these substituents represent alkyl groups. Those of R₁, R₂ and R₃ which represent alkyl groups may represent branched or straight chain saturated alkyl groups such as methyl, ethyl, or n- or iso- propyl, n-, sec- or tert- butyl groups or they may represent alkyl groups which contain one or more substituent groups such as hydroxyl, alkoxy, carboxy or amino groups such as 2, hydroxyethane groups or hydroxypropane groups. Particular amines which are useful in the composition of this invention include monomethylamine, dimethylamine, trimethylamine, monoethylamine, diethylamine, triethylamine, monopropylamine, dipropylamine, tripropylamine, monoethanolamine, diethanolamine and triethanolamine. The most preferred amine is triethanolamine. The amount of amine which is added to the rosin will be that which is required in order to produce the desired amount of amine salt. Where the product is to be used directly to provide both the rosin component and the amine salt component of the dispersion, the amount of amine which is added will normally be sufficient to neutralise from 1 to 20%, preferably from 3 to 6% of the acid groups present in the rosin. Where the rosin component and amine salt component are prepared separately, and subsequently mixed, the amount of amine salt will normally be such that the mixture comprises the same proportions of neutralised and nonneutralised rosin acids.

The co-reactant component of the dispersions of this invention may be of any of the aluminium salts known to be useful in the sizing of paper such as aluminium sulphate, paper maker's alum Al₂(SO₄)₃.18H₂O, polyaluminium chlorides such as those having the formula

Al(OH)ₓ(SO₄)_{y}Cl_{z}

wherein x has a value in the range 1.35 to 1.65, y has a value of from 0.08 to 0.15 and z has a value of 3-(x+y), or those having the formula:

Alₙ(OH)ₘCl₃ₙ₋ₘ

wherein n has a value of from 1 to 20, m is less than 3n and
is at least 2 and preferably at least 5.

A particular type of polyaluminium chloride which is useful in the dispersions of this invention are those described in European Patent Application 145686 and those produced by the processes described in European Patent Application 181847. Another type of useful polyaluminium chloride are the aluminium chlorohydrates having the formula:

Alₓ(OH)_{y}Cl_{z}

wherein x has a value of from 1 to 4, preferably a value of 1, y and z, which may be the same or different, have values of from 0.5 to 2.5 and the ratio y:z has a value in the range 5:1 to 1:5.

The preferred co-reactant for use in the compositions of the present invention are the aluminium chlorohydrates.

The dispersions of the present invention may be prepared by simple admixture of the components thereof or by using any of the conventional techniques of the art. In particular the dispersions may be prepared using the inversion technique.

The rosin, preferably a fortified rosin, optionally treated with para formaldehyde in the presence of a para toluene sulphonic acid to inhibit crystallisation, and optionally one which has been at least partially neutralised with an amine, may be melted and a stabilising agent or mixture of stabilising agents may then be added as a concentrated (e.g. 50% by weight solids) aqueous solution. Sufficient water is stirred in to form a creamy water-in-oil emulsion (e.g. 20 to 40% based on the weight of rosin). On dilution with water the emulsion inverts to provide a stable oil-in-water emulsion, typically having solids content of from 20% by weight up to the maximum achievable oil-in-water concentration (often about 80% by weight solids) and preferably from 30% to 40% by weight solids. The rosin content of the emulsion or dispersion usually contains at least 90% of unsaponified rosin acids. The emulsions may then be blended with an aqueous solution of one or more co-reactants.

The emulsions may be used for sizing paper, including alumed paper.

The rosin dispersions may be formulated so as to comprise other ingredients known in the art. In particular the dispersions may comprise one or more stabilisers. A variety of surface active agents or emulsifiers may be used to stabilise the dispersions either in admixture with one another or with other known emulsifying agents or in conjunction with other known auxiliary stabilising agents. A preferred class of auxiliary stabilising agents are the protective colloids such as casein and compositions comprising rosin, an amine salt of a rosin acid, a co-reactant and a protective colloid form a preferred aspect of this invention. Other compounds which may be used to stabilise the dispersions include starch derivatives, cellulose derivatives such as hydroxyethyl cellulose, or polymeric materials such as polyvinyl pyrolidone.

Anionic, non-ionic, amphoteric, or cationic surfactants may be utilised as stabilisers in the dispersions of this invention. In general we prefer to utilise anionic or non-ionic surfactants.

Examples of surface active agents which find use in the compositions of this invention include
(i) salt of sulphonic acids having the general formula:- where R' represents a hydrocarbon residue having from 4-18 carbon atoms, m is an integer having a value of 1 or 2, n is an integer having a value of 4 to 25, X represents a hydrogen atom or a hydroxyl group and M represents a monovalent cation and
(ii) salts of sulphuric acid half esters having the general formula:- wherein R² represents a hydrogen atom or an alkyl group having from 1 to 4 carbon atoms, A represents a straight chain or branch chain alkylene group having 2 or 3 carbon atoms, p is an integer having a value of from 4 to 25 and Q is a monovalent cation including all those compounds described in United States Patent 4309338.

Alkyl benzene sulphonates wherein the alkyl substituent comprises from 8 to 24 carbon atoms including all those compounds described in United States Patent 4157982.

Sulphosuccinate half esters of fortified rosin having the formula:-

H₍₃₋ₘ₎. R.[(CH₂CH₂O)ₙ -OC.C₂H₃SO₃Na. COONa]ₘ;

wherein R is a fortified rosin acid tricarboxylate group, m has an average value of from 1.5 to 3, and n has an average value from 4.5 to 25; including all those described in European Patent Application 159794.

Compounds having one of the formula:-
wherein R represents an alkyl group comprising from 4 to 18 carbon atoms and R' represents an alkyl or alkenyl group comprising from 4 to 18 carbon atoms and n is an integer having a value of from 4 to 25 including all those described in United States Patent 4199369.

Sulphosuccinate salts of ethylene oxide condensates having the general formula:-
wherein R represents an alkyl group comprising from 4 to 18 carbon atoms and n is an integer having a value of from 4 to 25; including all those compounds described in United States Patent 4203776.

Organic phosphate esters having the general formulae:-
wherein R represents an alkyl an alkyl phenol, alkenyl or alkaryl group comprising from 5 to 20 carbon atoms, n had a value of from 5 to 20 and X represents a monovalent cation or hydrogen.

Cationic resin dispersant systems may also be used to stabilise the rosin dispersion of this invention. Examples of suitable materials include water soluable polyaminopolyamide epichlorohydrin resins, water soluble alkylene polyamine epichlorohydrin resins or poly(diallyl-amine) epichlorohydrin resins.

A further type of compound which can usefully be incorporated into the dispersions of this invention is that comprising ammonia or an ammonium salt or a precursor thereof such as urea, a chemically modified urea or a precursor thereof. Examples of compounds which are useful in the compositions of this invention include urea, thiourea, biuret. melamine, water-soluble urea-formaldehyde and melamine formaldehyde resins and derivates or urea, especially those reaction products obtained by reacting urea with an acid selected from the group comprising sulphamic acid, phosphoric acid, trichloroacetic acid, nitric acid, sulphuric acid, hydrochloric acid, stearic acid and acetic acid as described in United States Patent 4022634 and 4093779, the reaction products of urea with a Lewis acid such a p-toluene sulphonic acid as described in United States Patent 4141750, the reaction products of urea and sulphamic acid such as are described in United States Patent 4025354 and the products obtained by the reaction of urea and formic acid as described in United States Patent 4437894.

The preferred sources of ammonia or ammonium salt for use in the compositions of the present invention are the products obtained by the reaction of urea with sulphamic acid including all those products which are described in United States Patent 4025354. These modified ureas may be produced by combining urea with sulphamic acid and water. Ideally, the parts by weight of water equal the parts by weight of urea plus sulphamic acid, although the urea may be treated with the sulfamic acid with more water or with little or no water. The urea-sulphamic acid solution may be heated to a temperature which causes a change in the pH for example to rise in the pH to at least about 7.5.

When little or no water is used the temperature affecting the pH may be higher. In the preferred embodiment, however, where a 50% water-50% urea sulphamic acid solution is used, a temperature of about 212° and 235°F, preferably about 215° to 230°F will increase the pH up to at least about 7.9. Generally, the solution boils at the temperature which changes the pH and heating should be continued until after boiling has stopped to effect an irreversible pH change. Although the pH range is an important measurement of reaction completion, a more important consideration is the acidity of the first stage product measured as parts of water (ppm). When the sulphamic acid is heated with the urea, undetermined reactions occur which not only raise the pH to a basic value, but also affect the acidity of the solution. The desired minimum acidity is at least 1,000 ppm, with a preferred minimum 4,300. The actual amount of sulphamic acid is probably at least about 0.1% by weight of urea, with preferred amounts ranging from about 0.2% to about 8.0%. The maximum amount of sulphamic acid needed would be 15 or at most 20% by weight of urea to achieve the desired results. It has been found that 5% sulphamic acid produces an acidity of about 86,000 ppm with a pH of between 7.9 and 8.3 when processed in a 50% water, 50% urea plus sulphamic acid solution. Accordingly, sulphamic acid at 0 25% by weight of urea produces a first stage product with an acidity of 4,300 ppm. As indicated, the amount of sulphamic acid added to the solution is not as important as its resulting acidity in defining the first stage product of the novel size composition of this embodiment.

In a preferred embodiment the proportion of ammonia or ammonia salt (or in the preferred embodiment the precursor thereof) to rosin or fortified rosin in the dispersions of this invention may be in the range 5 to 60% and preferably 10 to 35% by weight.

A further class of ingredients which may usefully be incorporated into the compositions of this invention are the synthetic sizes such as alkenyl succinic anhydrides and especially the alkyl ketene dimers. These reagents may be used as well as or as a partial replacement for the rosin sizes. In general the ratio of the weight of the rosin components to the synthetic size components will be in the range 2:1 to 5:1.

The novel dispersions will normally be formulated as relatively concentrated compositions which are diluted prior to their use in the sizing process. In general, the dispersions will comprise from 25 to 60% and more usually from 30 to 45% by weight of the combined weight of the rosin, amine salt and co-reactant.

The compositions of the invention my be employed as an internal size or as a surface size. Their use as an internal size forms a preferred aspect of the present invention. Internal sizing processes comprise the dilution of the concentrated composition with water and the addition of the diluted composition to a pulp suspension. The amount of size compositon employed is generally in the range 0.1 to 5.0% by weight of solids based on the weight of fibres in the pulp slurry.

The emulsions may be used for sizing paper, including alumed paper.

The emulsions may contain biocides such as bactericides, slimicides and/or fungicides or diluents such as wax.

The invention is illustrated by the following Examples:

### Example 1

### Preparation of a Fortified Rosin and a Dispersion of that Rosin

509 kg of modified tall oil rosin were prepared by reacting a 100 parts of tall oil rosin (ring and ball softening point = 60°C) with 0.1 parts of paratoluene sulphonic acid at a temperature of 165-175°C. After a 15 minute period 2½ parts of paraformaldehyde (82%) was added over a period of about one hour, maintaining a temperature of 165-175°C. To this was added 6 parts of maleic anhydride, this was again allowed to react over a period of one hour, after an initial exotherm the temperature was kept at 165-175°C. The rosin was tested for residual maleic anhydride, using a water wash through a toluene solution of the rosin product.

The fortified rosin was loaded into a one tonnne pot using an agitator speed of 300 rpm, water and 10 kg of triethanolamine was added both to cool and partially neutralise the rosin product.

When the temperature had dropped to below 100°C a solution comprising 10 kg of casein, 2 kg of borax and 60 kg of water at 89°C were added quickly to effect inversion.

After allowing to thicken for a period not exceeding 5 minutes the emulsion was diluted.

### Example 2

509 kg of a rosin product as produced in Example 1 were loaded into a one tonne pot using an agitator speed of 300 rpm, water and 10 kg of triethanolamine was added.

When the temperature had dropped below 100°C a solution comprising 7 kg casein, 1$\frac{\text{1}}{\text{2}}$ kg borax, 5 kg of an organic phosphate ester surfactant, as described previously, and 60 kg of water at 80°C were added quickly to effect inversion.

### Example 3

### Preparation of a modified urea

358 kg of urea was placed into a 2 tonne vessel capable of both stirring and heating the resulting solution. 600 kg of water was added. Heating and stirring was commenced. To this was added 18 kg of sulphamic acid. After a solution was achieved the acidity was measured and found to be 20,000 ppm.

After 1 1/4 hours of stirring and when boiling (103°C) had ceased the acidity was measured at 0 ppm.

### Example 4

### Preparation of a Rosin Dispersion Comprising a Co-Reactant

800 kg of the 30% rosin emulsion produced in Example 2 was placed into a 3 tonne production unit. To this was added 400 kg of a 30% urea solution. The stirrer was switched on at 3,000 rpm (Greaves mixer). To this was added quickly (1-5 secs) 160 kg of an aluminium chlorohydrate solution. An additional 640 kg of the aluminium chlorohydrate solution was added over a period of one minute. The stirrer was switched off and the product filtered through a 40 mesh filter basket.

### Example 5

A dispersion was produced using the ingredients and procedures described in Example 4, except a 30% Lewis acid reacted urea was substituted for the 30% urea solution.

### Example 6

A dispersion was produced using the ingredients and procedures described in Example 4, with the exception that no urea was added.

### Example 7

A dispersion was produced using the ingredients and procedures described in Example 4, except that a polyaluminium chloride was substituted for the aluminium chlorohydrate.

### Example 8

A dispersion was produced using the ingredients and procedures described in Example 4, except that aluminium sulphate (paper maker's alum) was substituted for the aluminium chlorohydrate.

### Example 9

A dispersion was produced using the ingredients and procedures described in Example 4, except that 50 mole % of the aluminium chlorohydrate was substituted with a polyaluminium chloride.

### Example 10

Sizing tests were carried out as follows:-
Bleached sulphite pulp was beaten to Schopper Reigler 40° at 2% consistency.

To 600 cc of this pulp was added 800 cc of water and sufficient sizing agent to give the level listed in Table II. This was mixed gently.

A further 1 litre of water was added and sufficient sulphuric (0.1N) acid to control the pH to 6.5 after 30 mins standing. Sheeets were prepared on a British standard sheet former. The wet sheets were blotted off the wire, pressed at 50 psi for 5 minutes and dried at 95°C for 4 minutes on a phototgraphic print drier. After overnight conditioning the sizing efficiency was assessed using the Cobb test (1 minute).

### External Sizing - Surface

(a) Waste furnishing Schopper Reigler = 40°
(b) 100 Gsm
(c) No additional flocculants added

| Product of Example | % Rosin/Fibre | 24 Hour conditioned cobb 60 seconds |
|---|---|---|
| 4 | 0.055 | 50 |
| | 0.075 | 19.4 |
| | 0.111 | 18.5 |
| | 0.222 | 17.8 |
| | 0.333 | 18.5 |

## Claims

1. A paper-sizing composition in the form of a preformed stable aqueous dispersion for subsequent use in a paper-sizing process, characterised in that the composition has the ability to size paper stock, sheet or web to an effective extent when brought into contact with the stock, sheet or web during the sizing process and comprises the material obtainable by addition of at least one aluminium compound to an aqueous dispersion comprising rosin size and an amine salt of a rosin acid.

2. A composition according to claim 1, wherein the amine salt of a rosin acid is the product of neutralisation with an amine of a component selected from rosin, fortified rosin, esterified rosin, disproportionated rosin and mixtures thereof.

3. A composition according to claim 1 or 2, wherein the amine salt of a rosin acid is added to a rosin dispersion comprising the rosin size component of the composition.

4. A composition according to claim 1 or 2, wherein the amine salt of a rosin acid is formed by the partial neutralisation of the acid content of the rosin size component of the composition.

5. A composition according to claim 2, wherein the rosin size component is a rosin derivative and the amine salt of a rosin acid is produced by neutralisation of the corresponding rosin acid prior to or after its conversion to a rosin derivative.

6. A composition according to any preceding claim, wherein the amine salt of a rosin acid is formed by neutralisation using an amine having the formula: wherein R₁, R₂ and R₃ are the same or different and each represents an alkyl, substituted alkyl, ankenyl or substituted alkenyl group comprising 1 to 4 carbon atoms, or a hydrogen atom, subject to the proviso that at least one of R₁, R₂ and R₃ is not a hydrogen atom.

7. A composition according to claim 6, wherein at least one of R₁, R₂ and R₃ is substituted.

8. A composition according to claim 7, wherein the substituent is hydroxyl, alkoxy, carboxy or amino.

9. A composition according to claim 8, wherein R₁, R₂ or R₃ is 2-hydroxyethyl or 2-hydroxypropyl.

10. A composition according to claim 6, wherein the amine is monomethylamine, dimethylamine, trimethylamine, monoethylamine, diethylamine, triethylamine, monopropylamine, dipropylamine, tripropylamine, monoethanolamine or diethanolamine.

11. A composition according to claim 6, wherein the amine is triethanolamine.

12. A composition according to any preceding claim, wherein the amine salt is present in an amount representing from 1% to 20% of neutralisation of the acid groups present in the rosin component.

13. A composition according to any preceding claim, wherein the aluminium compound is an aluminum salt.

14. A composition according to claim 13, wherein the aluminium salt is selected from aluminium sulphate, paper-maker's alum, and polyaluminium chlorides having the formula:
Al(OH)ₓ(SO₄)_{y}Cl_{z}
wherein x has a value in the range from 1.35 to 1.65, y has a value of from 0.08 to 0.15 and z has a value of 3-(x+y), or those having the formula;
Alₙ(OH)ₘCl₃ₙ₋ₘ
wherein n has a value of from 1 to 20, m is less than 3n and is at least 2.

15. A composition according to claim 13, wherein the aluminium salt is an aluminium chlorohydrate having the formula:
Alₓ(OH)_{y}Cl_{z}
wherein x has a value of from 1 to 4, preferably a value of 1 , y and z, which may be the same or different, have values of from 0.5 to 2.5 and the ratio y:z has a value in the range 5:1 to 1:5.

16. A composition according to any preceding claim, which has been prepared by an inversion technique.

17. A composition according to any preceding claim, wherein at least one stabiliser, optionally in conjunction with at least one auxiliary stabilising agent, is present.

18. A composition according to claim 17, wherein the stabiliser is selected from protective colloids, starch derivatives, cellulose derivatives, polymeric materials and anionic, nonionic, cationic and amphoteric surfactants, water-soluble polyaminopolyamide/epichlorohydrin resins, water-soluble alkylene-polyamine/epichlorohydrin resins and poly(diallylamine)/epichlorohydrin resins.

19. A composition according to any preceding claim, wherein ammonia, an ammonium salt or a precursor thereof is incorporated into the composition.

20. A composition according to any preceding claim, wherein at least one alkenyl succinic anhydride or alkyl ketene dimer synthetic size is incorporated into the composition.

21. A composition according to any preceding claim, which comprises from 25% to 60% by weight of the combined rosin component, co-reactant and amine salt.

22. A method of manufacture of a paper-sizing composition, the composition being characterized in that it is in the form of a stable aqueous dispersion for subsequent use in a paper-sizing process, and has the ability to size paper stock, sheet or web to an effective extent when brought into contact with the stock, sheet or web during the sizing process, the method comprising first forming an aqueous dispersion comprising rosin size and an amine salt of a rosin acid and then introducing at least one aluminium compound into the dispersion.

23. A method according to claim 22, wherein the amine salt is formed by addition of free amine to the rosin size to effect partial neutralisation of the rosin acid component of the rosin size.

24. A method according to claim 22, wherein the amine salt is formed separately and subsequently added as such to the rosin size.

25. A method according to claim 22, 23 or 24, wherein the amine salt of rosin acid is the salt of rosin acid and monomethylamine, dimethylamine, trimethylamine, monoethylamine, diethylamine, triethylamine, monopropylamine, dipropylamine, tripropylamine or diethanolamine.

26. A method according to claim 22, 23 or 24, wherein the amine salt of rosin acid is the salt of rosin acid and triethanolamine.

27. A method according to claim 22, wherein the aluminium compound is an aluminium salt selected from aluminium sulphate, paper-maker's alum, polyaluminium chlorides having the formula:
Al(OH)_{X}(SO₄)_{y}Cl_{z}
wherein x has a value in the range from 1.35 to 1.65, y has a value of from 0.08 to 0.15 and z has a value of 3-(x+y), or those having the formula:
Alₙ(OH)ₘCl₃ₙ₋ₘ
wherein n has a value of from 1 to 20, m is less than 3n and 3n-m/m is at least 2, and an aluminium chlorohydrate having the formula:
Alₓ(OH)_{y}Cl_{z}
wherein x has a value of from 1 to 4, preferably a value of 1, y and z, which may be the same or different, have values of from 0.5 to 2.5 and the ratio y:z has a value in the range 5:1 to 1:5.

28. A method according to any of claims 22 to 27, wherein a water-in-oil emulsion comprising the rosin component and at least one stabilizer is made and is then subjected to an inversion technique so as to form the desired composition in the form of an oil-in-water emulsion, which is then blended with at least one aluminium compound.

29. A process of manufacture of a sized paper product, wherein a paper-sizing composition is added to fibre stock which is then made into paper or is applied as a surface size to a prepared paper web or sheet, the composition being characterized in that it comprises the material obtainable by addition of at least one aluminium compound to an aqueous dispersion comprising rosin size and an amine salt of a rosin acid.

30. A process according to claim 29, wherein the composition is employed in an amount in the range from 0.1% to 5.0% by weight of solids based on the weight of the fibres in the pulp used to make the paper product.

31. A process according to claim 29 or 30, wherein the paper sizing composition is a composition according to any of claims 1 to 21.

## Patentansprüche

1. Papierleimungsmittel in Form einer vorgeformten stabilen wäßrigen Dispersion zur anschließenden Verwendung in einem Papierleimungsverfahren, dadurch gekennzeichnet, daß das Mittel die Fähigkeit besitzt Papierrohstoff, Papierbahnen oder auf Format geschnittenes Papier in einem wirksamen Ausmaß zu leimen, wenn es während des Leimungsverfahrens in Kontakt mit dem Papierrohstoff, den Papierbahnen oder dem auf Format geschnittenen Papier gebracht wird; und daß es das Material umfaßt, das durch Zugabe wenigstens einer Aluminiumverbindung zu einer einen Harzleim und ein Aminsalz einer Harzsäure umfassenden wäßrigen Dispersion, erhältlich ist.

2. Mittel gemäß Anspruch 1, wobei das Aminsalz einer Harzsäure das Produkt der Neutralisation einer Komponente, die ausgewählt ist aus Kolophonium, angereichertem Kolophonium, verestertem Kolophonium, disproportioniertem Kolophonium oder Gemischen davon, mit einem Amin ist.

3. Mittel gemäß Anspruch 1 oder 2, wobei das Aminsalz einer Harzsäure zu einer Kolophonium-Dispersion, die die Harzleimkomponente des Mittels umfaßt, hinzugefügt wird.

4. Mittel gemäß Anspruch 1 oder 2, wobei das Aminsalz einer Harzsäure durch teilweise Neutralisation des Säuregehalts der Harzleimkomponente des Mittels erzeugt wird.

5. Mittel gemäß Anspruch 2, wobei die Harzleimkomponente ein Kolophonium-Derivat ist, und das Aminsalz einer Harzsäure durch Neutralisation der entsprechenden Harzsäure vor oder nach deren Umwandlung in ein Kolophonium-Derivat hergestellt wird.

6. Mittel gemäß einem vorhergehenden Anspruch, wobei das Aminsalz der Harzsäure durch Neutralisation eines Amins der Formel erzeugt wird; in der die Reste R₁, R₂ und R₃ gleich oder verschieden sind und einen Alkyl-, substituierten Alkyl-, Alkenyl- oder substituierten Alkenylrest mit 1 bis 4 Kohlenstoffatomen, oder ein Wasserstoffatom darstellen, mit der Maßgabe, daß wenigstens einer der Reste R₁, R₂ und R₃ kein Wasserstoffatom ist.

7. Mittel gemäß Anspruch 6, wobei wenigstens einer der Reste R₁, R₂ und R₃ substituiert ist.

8. Mittel gemäß Anspruch 7, wobei der Substituent eine Hydroxy-, Alkoxy-, Carboxy- oder Aminogruppe ist.

9. Mittel gemäß Anspruch 8, wobei R₁, R₂ oder R₃ eine 2-Hydroxyethyl- oder eine 2-Hydroxypropylgruppe sind.

10. Mittel gemäß Anspruch 6, wobei das Amin Monomethylamin, Dimethylamin, Trimethylamin, Monoethylamin, Diethylamin, Triethylamin, Monopropylamin, Dipropylamin, Tripropylamin, Monoethanolamin oder Diethanolamin ist.

11. Mittel gemäß Anspruch 6, wobei das Amin Triethanolamin ist.

12. Mittel gemäß einem vorhergehenden Anspruch, wobei das Aminsalz in einer Menge vorhanden ist, die 1 bis 20 % Neutralisation der in der Kolophonium-Komponente vorhandenen Säuregruppen entspricht.

13. Mittel gemäß einem vorhergehenden Anspruch, wobei die Aluminiumverbindung ein Aluminiumsalz ist.

14. Mittel gemäß Anspruch 13, wobei das Aluminiumsalz ausgewählt ist aus Aluminiumsulfat, Papierherstellungs-Alaun und Polyaluminiumchloriden der Formel;
Al(OH)ₓ(SO₄)_{y}Cl_{z}
in der x einen Wert von 1,35 bis 1,65, y einen Wert von 0,08 bis 0,15 und z einen Wert von 3-(x+y) annimmt; oder solchen der Formel:
Alₙ(OH)ₘCl₃ₙ₋ₘ
in der n einen Wert von 1 bis 20 annimmt, m kleiner als 3n und 3n-m/m wenigstens 2 ist.

15. Mittel gemäß Anspruch 13, wobei das Aluminiumsalz ein Aluminiumchlorhydrat der Formel
Alₓ(OH)_{y}Cl_{z}
ist; in der x einen Wert von 1 bis 4, vorzugsweise 1 annimmt, y und z, die gleich oder verschieden sein können, Werte von 0,5 bis 2,5 annehmen und das Verhältnis y : z im Bereich 5:1 bis 1:5 liegt.

16. Mittel gemäß einem vorhergehenden Anspruch, das nach einer Inversionstechnik hergestellt wurde.

17. Mittel gemäß einem vorhergehenden Anspruch, in dem wenigstens ein Stabilisator, gegebenenfalls in Verbindung mit wenigstens einem Hilfsstabilisator, vorhanden ist.

18. Mittel gemäß Anspruch 17, wobei der Stabilisator ausgewählt ist aus Schutzkolloiden, Stärkederivaten, Cellulosederivaten, polymeren Stoffen sowie anionischen, nichtionischen, kationischen und amphoteren oberflächenaktiven Stoffen, wasserlöslichen Polyaminpolyamid/Epichlorhydrin-Harzen, wasserlöslichen Alkylenpolyamin/Epichlorhydrin-Harzen und Poly(diallylamin)/Epichlorhydrinharzen.

19. Mittel gemäß einem vorhergehenden Anspruch, wobei Ammoniak, ein Ammoniumsalz oder ein Vorläufer davon, in das Mittel eingearbeitet wird.

20. Mittel gemäß einem vorhergehenden Anspruch, wobei wenigstens ein synthetischer Leim, nämlich ein Alkenylbernsteinsäureanhydrid oder ein Alkylketendimeres, in das Mittel eingearbeitet wird.

21. Mittel gemäß einem vorhergehenden Anspruch, das 25 bis 60 Gew.-% der Kombination von Harzkomponente, Koreaktanten und Aminsalz umfaßt.

22. Verfahren zur Herstellung eines Papierleimungsmittels, das dadurch gekennzeichnet ist, daß es in Form einer stabilen wäßrigen Dispersion für die spätere Verwendung in einem Papierleimungsverfahren vorliegt, und daß es die Fähigkeit besitzt, Papierrohstoff, Papierbahnen und auf Format geschnittenes Papier in einem wirksamen Ausmaß zu leimen, wenn es während des Leimungsverfahrens in Kontakt mit dem Papierrohstoff, Papierbahnen oder auf Format geschnittenem Papier gebracht wird, wobei das Verfahren zuerst die Erzeugung einer wäßrigen Dispersion, die Harzleim und ein Aminsalz einer Harzsäure umfaßt, und dann das Einbringen wenigstens einer Aluminiumverbindung in die Dispersion umfaßt.

23. Verfahren gemäß Anspruch 22, wobei das Aminsalz sich bei der Addition des freien Amins zu dem Harzleim bildet, und eine teilweise Neutralisation der Harzsäurekomponente des Harzleims bewirkt.

24. Verfahren gemäß Anspruch 22, wobei das Aminsalz getrennt erzeugt und später als solches zum Harzleim hinzugefügt wird.

25. Verfahren gemäß den Ansprüchen 22, 23 oder 24, wobei das Aminsalz der Harzsäure das Salz der Harzsäure und von Monomethylamin, Dimethylamin, Trimethylamin, Monoethylamin, Diethylamin, Triethylamin, Monopropylamin, Dipropylamin, Tripropylamin oder Diethanolamin ist.

26. Verfahren gemäß den Ansprüchen 22, 23 oder 24, wobei das Aminsalz der Harzsäure das Salz der Harzsäure und von Triethanolamin ist.

27. Verfahren gemäß Anspruch 22, wobei die Aluminiumverbindung ein Aluminiumsalz ist, ausgewählt aus Aluminiumsulfat, Papierhrstellungs-Alaun und Polyaluminiumchloriden der Formel
Al(OH)ₓ(SO₄)_{y}Cl_{z}
in der x einen Wert von 1,35 bis 1,65, y einen Wert von 0,08 bis 0,15 und z einen Wert von 3-(x+y) annimmt; oder solchen der Formel:
Alₙ(OH)ₘCl₃ₙ₋ₘ
in der n einen Wert von 1 bis 20 annimmt, m kleiner als 3n und 3n-m/m wenigstens 2 ist; und einem Aluminiumchlorhydrat der Formel:
Alₓ(OH)_{y}Cl_{z}
in der x einen Wert von 1 bis 4, vorzugsweise 1 annimmt, y und z, die gleich oder verschieden sein können, Werte von 0,5 bis 2,5 annehmen und das Verhältnis y:z im Bereich 5:1 bis 1:5 liegt.

28. Verfahren gemäß einem der Ansprüche 22 bis 27, wobei eine Wasser-in-Öl-Emulsion, die die Harzkomponente und wenigstens einen Stabilisator umfaßt, hergestellt und anschließend einer Inversionstechnik ausgesetzt wird, so daß das gewünschte Mittel in Form einer Öl-in-Wasser-Emulsion erzeugt wird, die dann mit wenigstens einer Aluminiumverbindung gemischt wird.

29. Verfahren zur Herstellung eines geleimten Papierprodukts, wobei ein Papierleimungsmittel zu einem Papierfaserstoff hinzugefügt wird, der dann zu Papier verarbeitet wird, oder der als Oberflächenleim für hergestellte Papierbögen oder auf Format geschnittenes Papier verwendet wird, wobei das Mittel dadurch gekennzeichnet ist, daß es das Material umfaßt, das durch Zugabe wenigstens einer Aluminiumverbindung zu einer wäßrigen Dispersion, die Harzleim und ein Aminsalz der Harzsäure umfaßt, erhältlich ist.

30. Verfahren gemäß Anspruch 29, wobei das Mittel in einer Menge im Bereich von 0,1 bis 5,0 Gew.-% Feststoffe, bezogen auf die Masse des im Faserbrei enthaltenen Faserstoffs, aus dem das Papierprodukt hergestellt wird, angewendet wird.

31. Verfahren gemäß Anspruch 29 oder 30, wobei das Papierleimungsmittel ein Mittel gemäß den Ansprüchen 1 bis 21 ist.

## Revendications

1. Composition d'encollage de papier sous la forme d'une dispersion aqueuse stable formée préalablement, pour l'utilisation subséquente dans un procédé d'encollage de papier, caractérisée en ce que la composition présente l'aptitude à encoller la pâte à papier, la feuille ou le lai de papier dans une mesure efficace lorsqu'elle est mise en contact avec la pâte à papier, la feuille ou le lai de papier pendant l'opération d'encollage, et en ce qu'elle comprend la substance qui peut être obtenue par addition d'au moins un composé d'aluminium à une dispersion aqueuse comprenant un agent d'encollage à base de rosine et un sel d'amine d'un acide de rosine.

2. Composition selon la revendication 1, dans laquelle le sel d'amine d'un acide de rosine est le produit de neutralisation avec une amine d'un composant choisi parmi la rosine, la rosine renforcée, la rosine estérifiée, la rosine déproportionnée et leurs mélanges.

3. Composition selon la revendication 1 ou 2, dans laquelle le sel d'amine d'un acide de rosine est ajouté à une dispersion de rosine comprenant le composant d'encollage de rosine de la composition.

4. Composition selon la revendication 1 ou 2, dans laquelle le sel d'amine d'un acide de rosine est formé par la neutralisation partielle de la teneur en acide du composant agent d'encollage à base de rosine de la composition.

5. Composition selon la revendication 2, dans laquelle le composant agent d'encollage à base de rosine est un dérivé de rosine et le sel d'amine d'un acide de rosine est obtenu par neutralisation de l'acide de rosine correspondant avant ou après sa transformation en un dérivé de rosine.

6. Composition selon l'une quelconque des revendications précédentes, dans laquelle le sel d'amine d'un acide de rosine est formé par neutralisation à l'aide d'une amine répondant à la formule : dans laquelle R₁, R₂ et R₃ sont identiques ou différents et représentent chacun un groupe alkyle, alkyle substitué, alcényle ou alcényle substitué, comprenant 1 à 4 atomes de carbone, ou un atome d'hydrogène, étant entendu qu'au moins l'un de R₁, R₂ et R₃ ne représente pas un atome d'hydrogène.

7. Composition selon la revendication 6, dans laquelle au moins l'un de R₁, R₂ et R₃ est substitué.

8. Composition selon la revendication 7, dans laquelle le substituant est un groupe hydroxyle, alcoxy, carboxy ou amino.

9. Composition selon la revendication 8, dans laquelle R₁, R₂ ou R₃ représente un groupe 2-hydroxyéthyle ou 2-hydroxypropyle.

10. Composition selon la revendication 6, dans laquelle l'amine est la monométhylamine, la diméthylamine, la triméthylamine, la monoéthylamine, la diéthylamine, la triéthylamine, la monopropylamine, la dipropylamine, la tripropylamine, la monoéthanolamine ou la diéthanolamine.

11. Composition selon la revendication 6, dans laquelle l'amine est la triéthanolamine.

12. Composition selon l'une quelconque des revendications précédentes, dans laquelle le sel d'amine est présent en une quantité représentant 1 % à 20 % de la neutralisation des groupes acides présents dans le composant à base de rosine.

13. Composition selon l'une quelconque des revendications précédentes, dans laquelle le composé d'aluminium est un sel d'aluminium.

14. Composition selon la revendication 13, dans laquelle le sel d'aluminium est choisi parmi le sulfate d'aluminium, l'alun des papetiers et les poly(chlorure d'aluminium) répondant à la formule :
Al(OH)ₓ(SO₄)_{y}Cl_{z}
dans laquelle x a une valeur comprise dans la gamme de 1,35 à 1,65, y a une valeur comprise dans la gamme 0,08 à 0,15 et z vaut 3-(x+y), ou ceux répondant à la formule :
Alₙ(OH)ₘCl₃ₙ₋ₘ
dans laquelle n vaut de 1 à 20, m a une valeur inférieure à 3n et vaut au moins 2.

15. Composition selon la revendication 13, dans laquelle le sel d'aluminium est un chlorhydrate d'aluminium répondant à la formule :
Alₓ(OH)_{y}Cl_{z}
dans laquelle x vaut de 1 à 4, de préférence x vaut 1, y et z, qui peuvent être identiques ou différents, valent de 0,5 à 2,5, et le rapport y:z est dans la gamme de 5:1 à 1:5.

16. Composition selon l'une quelconque des revendications précédentes, qui a été préparée par une technique d'inversion.

17. Composition selon l'une quelconque des revendications précédentes, dans laquelle au moins un stabilisant est prévu, éventuellement conjointement avec au moins un agent stabilisant auxiliaire.

18. Composition selon la revendication 17, dans laquelle le stabilisant est choisi parmi les colloïdes protecteurs, les dérivés d'amidon, les dérivés cellulosiques, les substances polymères et les tensioactifs anioniques, non ioniques, cationiques et amphotères, les résines polyaminopolyamide/épichlorhydrine hydrosolubles, les résines alkylène-polyamine/épichlorhydrine hydrosolubles et les résines poly(diallylamine)/épichlorhydrine.

19. Composition selon l'une quelconque des revendications précédentes, dans laquelle de l'ammoniac, un sel d'ammonium ou un de ses précurseurs est incorporé dans la composition.

20. Composition selon l'une quelconque des revendications précédentes, dans laquelle au moins un agent d'encollage de synthèse anhydride alcénylsuccinique ou dimère d'alkylcétène est incorporé dans la composition.

21. Composition selon l'une quelconque des revendications précédentes, qui comprend 25 % à 60 % en poids du composé à base de résine, du co-réactant et du sel d'amine combinés.

22. Procédé de fabrication d'une composition d'agent d'encollage de papier, la composition étant caractérisée en ce qu'elle est sous la forme d'une dispersion aqueuse stable pour l'utilisation subséquente dans un procédé d'encollage de papier, et présente l'aptitude à encoller la pâte à papier, la feuille ou le lai de papier dans une mesure efficace lorsqu'elle est mise en contact avec la pâte à papier, la feuille ou le lai de papier pendant le procédé d'encollage, le procédé comprenant d'abord la formation d'une dispersion aqueuse comprenant l'agent d'encollage à base de rosine et un sel d'amine d'un acide de rosine, et ensuite, l'introduction dans la dispersion d'au moins un composé d'aluminium.

23. Procédé selon la revendication 22, dans lequel le sel d'amine est formé par addition d'une amine libre à l'agent d'encollage à base de rosine pour effectuer la neutralisation partielle du composant acide de rosine de l'agent d'encollage à base de rosine.

24. Procédé selon la revendication 22, dans lequel le sel d'amine est formé séparément et ajouté subséquemment tel quel à l'agent d'encollage à base de rosine.

25. Procédé selon la revendication 22, 23 ou 24, dans lequel le sel d'amine de l'acide de rosine est le sel de l'acide de rosine et de monométhylamine, diméthylamine, triméthylamine, monoéthylamine, diéthylamine, triéthylamine, monopropylamine, dipropylamine, tripropylamine ou diéthanolamine.

26. Procédé selon la revendication 22, 23 ou 24, dans lequel le sel d'amine de l'acide de rosine est le sel d'acide de rosine et de triéthanolamine.

27. Procédé selon la revendication 22, dans lequel le composé d'aluminium est un sel d'aluminium choisi parmi le sulfate d'aluminium, l'alun des fabricants de papier, les poly(chlorure d'aluminium) répondant à la formule :
Al(OH)ₓ(SO₄)_{y}Cl_{z}
dans laquelle x a une valeur comprise dans la gamme de 1,35 à 1,65, y a une valeur comprise dans la gamme de 0,08 à 0,15 et z vaut 3-(x+y), ou ceux répondant à la formule :
Alₙ(OH)ₘCl₃ₙ₋ₘ
dans laquelle n vaut de 1 à 20, m a une valeur inférieure à 3n et vaut au moins 2, et un chlorhydrate d'aluminium répondant à la formule :
Alₓ(OH)_{y}Cl_{z}
dans laquelle x vaut de 1 à 4, de préférence 1, y et z, qui peuvent être identiques ou différents, valent de 0,5 à 2,5, et le rapport y:z présente une valeur dans la gamme de 5:1 à 1:5.

28. Procédé selon l'une quelconque des revendications 22 à 27, dans lequel une émulsion eau-dans-huile comprenant le composant de rosine et au moins un stabilisant est préparé, et est ensuite soumise à une technique d'inversion de façon à former la composition voulue sous la forme d'une émulsion huile-dans-eau, qui est ensuite mélangée avec au moins un composé d'aluminium.

29. Procédé de fabrication d'un produit papetier encollé, dans lequel une composition d'encollage de papier est ajoutée à une pâte à papier qui est ensuite transformée en papier, ou est appliquée comme agent d'encollage de surface sur une feuille ou un lai de papier préparé, la composition étant caractérisée en ce qu'elle comprend la substance qui peut être obtenue par addition d'au moins un composé d'aluminium à une dispersion aqueuse comprenant un agent d'encollage à base de rosine et un sel d'amine d'un acide de rosine.

30. Procédé selon la revendication 29, dans lequel la composition est utilisée en une quantité comprise entre 0,1 % et 5,0 % en poids de substances solides, par rapport au poids des fibres contenus dans la pâte utilisée pour fabriquer le produit papetier.

31. Procédé selon la revendication 29 ou 30, dans lequel la composition d'encollage du papier est une composition selon l'une quelconque des revendications 1 à 21.
